

## UNITED STATES PATENT OFFICE

1,968,140

## PLASTIC WAX BOARD LINER

Daniel M. Gray, Wheeling, W. Va., assignor to  
 Hazel-Atlas Glass Co., Wheeling, W. Va., a corporation of West Virginia

No Drawing. Application June 10, 1930,  
 Serial No. 460,298

2 Claims. (Cl. 215—38)

This invention relates to liners for bottle and jar closures and has special reference to liners which are commonly known to the trade as a plastic wax board liner.

5 Liners of this type are highly desirable for the packaging of certain classes of goods in glass containers, but as now constructed are comparatively expensive in that the wax coating comprises, among other constituents, ceresin and 60 bees wax. It is the primary object of the present invention therefore, to provide a wax board liner of low cost and yet which will have all of the salient features of the more expensive liner.

15 I have found from a long series of experiments that when crude rubber is dissolved in molten paraffin wax for a short time at low temperature, a viscous mixture results, which when applied to pulp board or the like, and cooled, provides an excellent wax board liner.

20 The experimentation has been carried out with a variety of grades of crude rubber, and while practically all are found to be suitable for dissolving in paraffin and for imparting the desired plasticity to the resulting mixture, best results 65 have been obtained when using pale crepe plantation rubber of a type having a minimum amount of the rubber odor. Various percentages of crude rubber and paraffin have been tested, and while plastic compositions of good quality have resulted 70 in most instances, it is found that a compound containing 12% to 14% of crude rubber by weight and about 88% to 86% of paraffin is the most desirable in practice.

35 In manufacturing the improved liner the paraffin is first melted and the desired percentage of rubber (preferably pale crepe plantation rubber) added. The temperature at which the paraffin is melted should be maintained as low as possible 75 and only for such length of time as is necessary to obtain a complete solution of the rubber. This is of paramount importance for the reason that it has been found that prolonged heating of the mixture, or too high temperatures, results in a lowering of the viscosity of the mixture. Where- 80 as a mixture of fairly high viscosity is desirable

for use as a coating for liners; otherwise the mixture will impregnate the pulp board, with a consequent increase in the cost of manufacture.

The pulp board or other material employed as a base for the liners is coated with the comparatively thick and viscous mixture of paraffin and rubber, by dipping or otherwise, and the coated material is then allowed to cool or may be cooled artificially. A uniform and unbroken film of the wax mixture is thus formed on the board; and to 85 complete the liner it is only necessary that discs of the desired diameter be stamped out in the usual way.

Liners of pulp board or the like, coated with a wax-rubber mixture as above described, are 90 found to be highly efficient in use, are practically free from objectionable odor, and are, of course, considerably cheaper to manufacture than the wax board liners now in use.

95 While in describing the invention I have referred specifically to pulp board and paraffin, it is to be understood that other waxes may be substituted for paraffin in the mixture and that other material such as paper or the like, may be used 75 in lieu of pulp board.

In accordance with the patent statutes I have described what I now believe to be the preferred form of the invention, but the percentages of materials used in the mixture as well as the manner of its preparation and application may vary 80 considerably, and all such variations are intended to be included within the scope of the appended 85 claims.

What I claim is:

1. A liner for jar closures comprising a body 90 of pulp board, said body coated with a plastic mixture composed of approximately 88% paraffin and approximately 12% rubber.

2. A liner for jar closures comprising a body of 95 pulp board, said body coated with an unbroken film of a plastic mixture composed of approximately 88% paraffin and approximately 12% pale crepe plantation rubber.

DANIEL M. GRAY.

100